

# UNITED STATES PATENT OFFICE.

ARTHUR GEORGE MUMFORD, OF COLCHESTER, ENGLAND.

## METHOD OF MAKING ALLOYS.

1,355,769.

Specification of Letters Patent. Patented Oct. 12, 1920.

No Drawing.

Application filed January 26, 1920. Serial No. 354,240.

*To all whom it may concern:*

Be it known that I, ARTHUR GEORGE MUMFORD, a subject of the King of Great Britain and Ireland, residing at the Culver Street 5 Engineering Works, Colchester, in the county of Essex, England, director of public company, have invented a new and useful Improvement in Methods of Making Alloys, of which the following is a specification.

10

This invention relates to an improved method of making alloys of copper containing fractional percentages of tin and zinc and it has for its object generally to make 15 reliable castings for floats for automatic feed water regulators and the like which are subjected to very high temperatures and pressures and a constant variation of same and which will not become water logged 20 and specifically to so mix the small percentage of zinc, which is a highly volatile metal, with the other metals that the percentage of same can be insured with a reasonable degree of accuracy.

A suitable alloy for the purpose comprises 86.168% of copper, 11.97% of tin and 1.842% of zinc. 25

In making this alloy a white metal alloy composed of 61% of tin, 29.7% of copper and 9.3% of zinc is first made and run into 30 an ingot, and then the final alloy is made of 80.36% of copper and 19.64% of the aforesaid white metal alloy.

Castings of this alloy are made in iron 35 chills and have the characteristics that they are homogeneous, non-absorbent and will stand both high temperatures and high pressure and continual variations of same.

I claim:

The improved method of making an alloy 40 of copper, tin and zinc consisting in first making an alloy of these metals in the following proportions:—tin 61%, copper 29.7% and zinc 9.3%, and then making the final alloy of 19.64% of said white metal alloy 45 and 80.36% of copper.

ARTHUR GEORGE MUMFORD.